

# UNITED STATES PATENT OFFICE.

HERMANN HILBERT, OF HEUFELD, GERMANY.

## MANUFACTURE OF GELATIN AND GLUE FROM BONES.

No 834,806.

Specification of Letters Patent.

Patented Oct. 30, 1906.

Application filed June 7, 1904. Serial No. 211,550.

To all whom it may concern:

Be it known that I, HERMANN HILBERT, Ph. D., chemist, of Heufeld, Upper Bavaria, in the German Empire, have invented a new and useful Improvement in the Manufacture of Gelatin and Glue from Bones, of which the following is a specification.

The process is essentially as follows: The bones are ground to a fine flour and introduced into a vessel which is fitted with a stirring apparatus. In this apparatus the powdered bones are boiled with water while being stirred, and at the same time while the glue is being extracted sulfurous-acid gas or other bleaching agents, such as sulfites and bisulfites, with other acids or with other sulfurous or hydrosulfurous compounds, nascent hydrogen, hydrogen peroxid, and the like, are introduced. In this process the glue, which goes quickly into the solution, is bleached at the moment in which it is dissolving. In the same moment the sulfurous acid is used up, so that there is no excess which can spoil the glue solution. As this glue-extracting process takes place very quickly, the bleaching process also is finished in the same short time, so that no glue is wasted and the glue remains of a very superior quality. Moreover, the process possesses the very great advantage that the extracting of the glue takes place at a temperature which is substantially much lower than is the case with processes as hitherto ordinarily employed, which exert a very important influence on the quality of the product.

The improved process may conveniently be carried out in practice in the following manner: In a suitable boiler containing water and most advantageously furnished with a stirring appliance the bone-flour is introduced and steam is admitted. At the same time the introduction of the bleaching agent is commenced. The carbon dioxid which is produced when acids are employed is led off and the glue or gelatin is gradually extracted from the bone-flour by boiling at atmospheric or higher pressure. The residual bone-flour is then separated from the liquor by filtration or by other known means.

Should the output not be satisfactory, the process may be repeated with the residual flour.

The above-described process has the following among other advantages: The extraction of the glue or gelatin may be effected at the boiling-point. The quality of the product is greatly improved. An almost absolutely colorless product can be obtained from common bones. Nearly the whole of the gelatin contained in the bones is recovered. The duration of the process is very short, so that the glue or gelatin is not damaged by the action of the bleaching agent or by prolonged boiling.

What I claim is—

1. The herein-described process of treating bones with bleaching agents during boiling bones for manufacturing glue and gelatin which consists in gradually adding the bleaching agent to the bones having been ground in the known manner to a flour.

2. The herein-described process of treating bones with bleaching agents during boiling the bones for manufacturing glue and gelatin which consists in gradually adding to the bones having been ground in the known manner to a flour the bleaching agent in such a manner that it is used up at the moment in which the glue is dissolving.

3. The herein-described process of treating bones with bleaching agents as sulfurous acid during boiling the bones for manufacturing glue and gelatin which consists in gradually adding the sulfurous acid to the bones having been ground in a known manner to a flour.

4. The herein-described process of treating bones with bleaching agents as sulfurous acid during boiling the bones for manufacturing glue and gelatin which consists in gradually adding to the bones having been ground in the usual manner to a flour the sulfurous acid in such a manner that it is used up at the moment in which the glue is dissolving.

In witness whereof I have hereunto set my hand in presence of two witnesses.

HERMANN HILBERT.

Witnesses:

C. HENRY, Elder,  
ULYSES J. BYWATER.